

# United States Patent Office

2,796,401

Patented June 18, 1957

1

2,796,401

## COMPLEX FORMAL LUBRICATING COMPOSITION

Alfred H. Matuszak, Westfield, William E. McTurk, Elizabeth, Delmer L. Cottle, Highland Park, and David W. Young, Westfield, N. J., assignors to Esso Research and Engineering Company, a corporation of Delaware

No Drawing. Application November 29, 1952,  
Serial No. 323,338

11 Claims. (Cl. 252—42)

This invention relates to synthetic lubricating compositions. Particularly the invention relates to synthetic lubricating compositions having outstanding lubricating properties at both high and low temperatures and which have the advantage of leaving substantially no combustion chamber deposits in the cylinders of reciprocating engines. More particularly the invention relates to new and improved synthetic lubricating oils which comprise the formals of organic compounds having at least one free hydroxyl group which is alcoholic in nature, and which contain a  $-\text{O}[\text{CH}_2-\text{O}(\text{C}_n\text{H}_{2n}\text{O})_y]_x\text{CH}_2-\text{O}-$  linkage,  $x$  and  $n$  being 2 or more and  $y$  being 1 or more.

In recent efforts to obtain superior lubricating compositions which have unusual and specific properties, there have been developed entirely new synthetic materials with lubricating properties. In general these new synthetic lubricants are characterized by viscosity properties that are outstanding at both low and high temperatures, especially when compared to mineral oils. These outstanding low and high temperature properties are especially desirable for use in equipment designed to operate over a great temperature differential, such as jet engines for aircraft use, combustion engines for aircraft, and the like. It has been found that mineral lubricating oils are generally undesirable for the lubricating of these engines because of their high and low temperature viscosity limitations.

It has also been found that synthetic lubricants may be desirable for the lubricating of standard automotive engines. In addition to the versatility of their viscosities, the use of some types of the synthetic lubricants investigated have been found to result in very low rates of combustion chamber deposit formation, particularly when used for long periods of time. Low rates of formation of combustion chamber deposits result in increased power factor from fuel, less increase in the octane requirement of the engine, less pre-ignition tendency, and a general overall improvement in engine operation. These new lubricants may also serve to reduce or remove combustion chamber deposits from an engine already loaded with such deposits.

The present invention relates to a new type of synthetic lubricating composition which comprises the formals of a wide range of organic compounds which contain at least one free hydroxyl group and which is alcoholic in nature and which contains at least three  $-\text{CH}_2\text{O}-$  linkages.

It has been generally accepted by the art that most acetals are not of sufficient stability to serve as lubricating compositions. It has now been found, however, and forms the object of this invention, that the formals of organic hydroxy compounds that contain the linkage  $-\text{O}[\text{CH}_2-\text{O}(\text{C}_n\text{H}_{2n}\text{O})_y]_x\text{CH}_2-\text{O}-$  where  $x$  and  $n$  are 2 or more and  $y$  is 1 or more have excellent stability and have viscosity properties that make them outstanding lubricating compositions.

A generic formula for the lubricating compositions of this invention may be written as follows:

2

$\text{A}-\text{O}[\text{CH}_2-\text{O}(\text{C}_n\text{H}_{2n}\text{O})_y]_x\text{CH}_2-\text{O}-\text{B}$

In the formula A and B represent the organic compounds less the hydroxyl group.  $x$  and  $n$  represent numbers having a value of 2 or more and  $y$  is 1 or more. The radicals 5 may be alike or different and may contain from 1 to 60 carbon atoms. A and B are selected such that the total number of carbon atoms in the formal is between about 20 and 130, with compounds containing from about 25 to 100 carbon atoms being preferred. The organic hydroxy compounds which serve as a source for the radicals A and B will be defined more in detail below.

For use in reciprocating engines, particularly as a lubricant for automotive engines, a lubricating composition 10 must meet several requirements. In order to form an effective lubricating film and to maintain that film at low and high temperatures it must have certain viscosity characteristics. At low temperatures the lubricant must be sufficiently labile to flow through the circulatory system of the equipment and allow movement of lubricated surfaces without an undue power requirement. A lubricant having an ASTM pour point below about 35° F. has sufficient low temperature lability to make it satisfactory in these respects for general use. At high temperatures a lubricant must have sufficient "body" or "thickness" to furnish and maintain a satisfactory lubricating film. It has been found that a lubricant that is satisfactory in this respect will have a viscosity at 210° F. of between about 2 to 60 centistokes, i. e. 32.8 and 280 Saybolt seconds, Universal. To prevent undue lubricant loss, due to volatility and general molecular disintegration and to insure against explosion hazards at higher temperatures sometimes encountered, a lubricating composition should have a flash point in excess of about 300° F. These requisites are inherent in the term "lubricating compositions," as used in this specification, and the formals of this invention are limited to those within these operable ranges. The preferred materials, as contemplated herein and as described in the preferred embodiment hereof, will have an ASTM pour point below about 40 45° F., a flash point above about 375° F., and will have a viscosity within the range of 2.6 to 13 centistokes, i. e., 35 to 70 Saybolt seconds, Universal, at 210° F.

In general it has been found that the above listed 45 properties are a function both of molecular structure and of molecular weight. This fact makes it possible, within certain limits, to prepare compositions having similar low and high temperature properties in a variety of ways and also enables the manufacturer to "tailor" a composition to fit a certain set of specifications within 50 rather general limits. This fact also accounts for the large number of organic materials containing alcoholic hydroxyl groups available for preparing the compositions of this invention.

In general the preparation of the complex formals of 55 this invention is accomplished by methods that require conventional techniques and methods. Three general lines of approach may be followed.

1. The reactants may be admixed in the reacting zone and heated to reflux temperature in the presence of an entraining agent such as hexane, heptane or the like. After recovery of the water of theory the product is washed free of any acidic catalysts and stripped free of unreacted components.

60 2. A second approach is to admix  $x$  moles of the glycol reactant with  $x-1$  moles of formaldehyde to obtain the central portion of the complex formal, i. e., the portion represented by  $\text{HO}(\text{C}_n\text{H}_{2n}\text{O})_y[\text{CH}_2-\text{O}-(\text{C}_n\text{H}_{2n}\text{O})]_x\text{H}$ . In another reacting zone equal moles of an alcohol and formaldehyde are heated to about 60° C. to obtain the hemiformal of the alcohol, i. e.,  $\text{R}-\text{O}-\text{CH}_2-\text{OH}$ . The materials are then blended by adding the glycol formal 65 70

to the alcohol hemiformal and heated to reflux temperature. The product, after removal of the theoretical water, is then washed and stripped as above.

3. In this third approach the hemiformal of the chosen alcohol is first made by heating equal moles of the alcohol and formaldehyde. Then to this is added the desired molar proportion of a glycol and formaldehyde and the total mixture heated to reflux temperature to make the hydroxy complex represented by



10

Two moles of this material is then reacted with one mole of formaldehyde to obtain the product which is purified as above.

The materials used to prepare these formals, that is 15 organic hydroxy compounds containing at least one free hydroxyl group which is alcoholic in character, may be selected from the following partial list. Others, of course, may be used.

20

I. Unsubstituted alcohols

A. Monohydric

1. Aliphatic

- (a) Methyl alcohol
- (b) Ethyl alcohol
- (c) Propyl alcohol
- (d) Isopropyl alcohol
- (e) n-Butyl alcohol
- (f) Iso-butyl alcohol
- (g) Sec.-butyl alcohol
- (h) Tert.-butyl alcohol
- (i) n-Amyl alcohol
- (j) Iso-amyl alcohol
- (k) n-Hexyl alcohol
- (l) Iso-hexyl alcohol
- (m) 2-ethyl-1-butanol
- (n) 2-ethyl-1-hexanol
- (o) Octyl alcohol
- (p) Iso-octyl alcohol
- (q) 2-octyl alcohol
- (r) Iso-nonyl alcohol
- (s) Decyl alcohol
- (t) Lauryl alcohol
- (u) Tetradecyl alcohol
- (v) Pentadecyl alcohol
- (w) Octadecyl alcohol
- (x) Allyl alcohol
- (y) Crotyl alcohol
- (z) Oleyl alcohol
- (aa) The terpineols
- (bb) C<sub>8</sub> to C<sub>20</sub> Oxo alcohols
- (cc) Alcohols derived from the "Synol" process
- (dd) Alcohols derived from the oxidation of petroleum fractions
- (ee) Alcohols derived from Guerbet's reaction
- (ff) Alcohols derived from the hydration of olefins
- (gg) Alcohols derived from the "Oxyl" synthesis
- (hh) Mixtures of the above

2. Aromatic

- (a) Benzyl alcohol
- (b) Phenethyl alcohol
- (c) 3-phenyl-1-propanol
- (d)  $\alpha$ -Naphthyl carbinol
- (e) Cinnamyl alcohol
- (f) Diphenyl carbinol
- (g) Furfuryl alcohol
- (h) Cumaric alcohol
- (i) Vanillyl alcohol
- (j) Piperonyl alcohol

B. Polyhydric

1. Glycols

- (a) Ethylene glycol
- (b) 1,2-propanediol
- (c) 1,3-propanediol
- (d) 1,3-butanediol
- (e) 1,4-butanediol
- (f) 1,5-pentanediol
- (g) The various polyalkylene glycols, e. g.
  - 1. Polyethylene glycols
    - (a) Diethylene glycol
    - (b) Triethylene glycol
    - (c) Tetraethylene glycol
  - 2. Polypropylene glycols
    - (a) Dipropylene glycol
    - (b) Tripropylene glycol
- (h) 1,2-cyclohexanediol
- (i) Decanediol-1,10

2. Other polyhydric alcohols

- (a) Glycerol
- (b) 2-hydroxymethyl-2-methyl-propanediol-1,3
- (c) Pentaerythritol
- (d) Sorbitol
- (e) Dipentaerythritol
- (f) Dulcitol
- (g) Trimethylol propane
- (h) Tetramethylol cyclohexanol
- (i) Benzotrimethylol

II. Substituted alcohols

A. Monohydric

1. Aliphatic

- (a) Halogenated alcohols
  - 1. Ethylene chlorohydrin

- 2. Trifluoro ethanol
- 3. Propylene chlorohydrin
- 4. The various chloro-substituted monoethers of polyalkylene glycols

- (b) Ethanolamine
- (c) 2-amino propanol
- (d) 2-nitroethanol
- (e) 2-nitropropanol
- (f) 2-nitrobutanol
- (g) The various glycol monoesters, e. g.

- 1. Ethylene glycol monoacetate
- 2. Propylene glycol monobutyrate
- 3. Butylene glycol monolaurate
- 4. Polyethylene glycol monoesters
- 5. Polypropylene glycol monoesters
- 6. Polybutylene glycol monoesters

- (h) The various glycol monoethers, e. g.
- 1. Ethylene glycol mono-methyl ether
- 2. Propylene glycol mono-butyl ether
- 3. Butylene glycol mono-lauryl ether
- 4. Polyethylene glycol mono-ethers
- 5. Polypropylene glycol mono-ethers
- 6. Polybutylene glycol mono-ethers
- 7. Polytrimethylene glycol mono-ethers

- (i) The various glycol mono-formals, e. g. the mixed formals of glycols and alcohols

- (j) Hydroxy alkyl cyanides
- 1. Ethylene cyanohydrin
- 2.  $\alpha$ -Hydroxy isobutyronitrile

- (k) Ethanol morpholine

2. Aromatic

- (a) p-Methoxy benzyl alcohol
- (b) The various chlorobenzyl alcohols
- (c) The various nitrobenzyl alcohols
- (d) 2-anilino ethanol

B. Polyhydric

1. Glycols

- (a) Halogenated glycols, e. g.
- 1. 3-chloro-1,2-propanediol
- 2. 2-chloro-1,3-propanediol

(b) Nitroglycols, e. g.

- 1. 2-nitro-1,3-propanediol
- 2. 2-nitro-2-methyl-propanediol-1,3
- 3. Trimethylol nitromethane

(c) Amino glycols

- 1. 2-amino-1,3-propanediol
- 2. 2-amino-2-methyl-1,3-propanediol
- 3. Diethanol amine
- 4. Trimethylol aminomethane

C. Other hydroxy compounds

- 1. Esters of hydroxy acids
- (a) The various lactate esters
- (b) The various glycolate esters
- (c) The various hydroxy stearate esters

2. Carboxy substituted alcohols

- (a) Hydroxy ketones, e. g.
- 1. Hydroxy acetone
- (b) Hydroxy aldehydes, e. g.
- 1.  $\alpha$ -Hydroxy adipaldehyde
- 2.  $\beta$ -Hydroxy propionaldehyde

Particularly desirable organic hydroxy compounds for use in this invention are those highly branched chain aliphatic alcohols prepared by the "Oxo" synthesis. This "Oxo" synthesis may be described as being the catalytic reaction of an olefin with carbon monoxide and hydrogen. The reaction occurs at temperatures in the order of 300°-400° F., at pressures in the range of about 1000 to 3000 p. s. i., in the presence of a suitable catalyst, ordinarily a heavy metal carbonyl such as cobalt carbonyl. The resulting aldehyde is subsequently hydrogenated to a primary alcohol. This process is described in U. S. Patent No. 2,327,066 issued to Roelen in 1943.

In general the oxygenated group in a product from an olefin by the Oxo process is thought of as becoming attached to an unsaturated carbon which holds at least one hydrogen atom. In those cases where the carbon monoxide attacks a "saturated" carbon atom, it must be assumed either that that carbon has become unsaturated prior to reaction by a shift of a hydrogen atom or that the attack is directly on a carbon atom that is truly saturated. For example, 2-butene has been reported to give 1-pentanol and 2-methylbutanol in equal quantities, a result that cannot be explained on the simple basis that oxonation takes place only on unsaturated carbons holding hydrogen. 2,3-dimethyl-2-butene also reacts giving only 3,4-dimethyl-1-pentanol; in this olefin no hydrogen is attached to the unsaturated carbon atoms and the attack of carbon monoxide must either be on a "rearranged" olefin or on a saturated carbon atom.

It has been found that particularly desirable alcohols for the formation of the formals of this invention can be prepared by the application of the Oxo synthesis to polymers and copolymers of C<sub>3</sub> and C<sub>4</sub> monoolefins. These monoolefins are readily available in petroleum

refinery streams and processes for their conversion to liquid copolymers have been worked out by the art. One such process, known as U. O. P. polymerization, consists of passing the olefin-containing stream in liquid phase in contact with an acid catalyst comprising phosphoric acid impregnated on kieselguhr. Other acidic catalysts, such as phosphoric acid or copper phosphate impregnated on silica gel, sulfuric acid, Friedel-Crafts catalysts, activated clays, silica-alumina, copper pyrophosphate, etc., may be used. Suitable conditions when employing phosphoric acid catalysts of the U. O. P. type are temperatures of 300° F. to 500° F., pressures from 250 to 5,000 p. s. i. and feed stocks comprising refinery streams containing propylene and mixed butylenes. Suitable feed stocks, for example, may contain from 15 to 60 mol percent propylenes, from 0.5 to 15 mol percent butylenes, and from 0.1 to 10 mol percent isobutylene, the remaining being saturated hydrocarbons. Other suitable feed stocks are the dimer and trimer of isobutylene.

The preferred Oxo alcohols employed in forming the formals of this invention are those having from 8 to 20 carbon atoms derived from olefin copolymers having from 7 to 19 carbon atoms. In preparing these Oxo alcohols the desired olefin fraction is segregated from the crude olefin polymer product by fractionation.

The following table, for example, shows the structure and percent composition of C<sub>8</sub> Oxo alcohols prepared from a C<sub>7</sub> olefin stream which had been fractionated from the products obtained by the phosphoric acid polymerization of refinery gas streams containing propylene and mixed n- and isobutylenes.

| Structure of C <sub>8</sub> Oxo Alcohols Prepared from C <sub>8</sub> -C <sub>4</sub> Copolymer Heptenes | Percent |
|----------------------------------------------------------------------------------------------------------|---------|
|                                                                                                          | 29      |
|                                                                                                          | 25      |
|                                                                                                          | 17      |
|                                                                                                          | 16      |
|                                                                                                          | 2.3     |
|                                                                                                          | 1.4     |
|                                                                                                          | 4.3     |
|                                                                                                          | 5.0     |
|                                                                                                          | 100.0   |

As was stated above, the formals of this invention, hereinafter referred to as complex formals, may be considered to have the following general formula:



In the formula A and B represent radicals derived from organic compounds by removal of one reacting hydroxyl group. In the formula x and n are 2 or more and y is one or more. The radicals represented by A and B may be alike or different and may contain from 1 to 60 carbon atoms. The sum of the carbon atoms in the molecule should be between 20 and 130 and preferably between about 25 and 100.

The group of organic compounds that satisfy the conditions of the above generic formula and that are used to build the preferred compounds according to the concept of this invention are monohydric alcohols, glycols, and organic acids. These compounds may be advantageously combined with formaldehyde to form molecules having the following type formulas, words instead of structures being given to show the components of the complex formals.

- 10      Alcohol-(formaldehyde-glycol)<sub>x</sub>  
 Glycol-(formaldehyde-glycol)<sub>x</sub>  
 Glycol monoester-(formaldehyde-glycol)<sub>x</sub>  
 Glycol monoether-(formaldehyde-glycol)<sub>x</sub>

15      In all formulas given above x represents a whole number greater than 1. The acids which may be used to prepare the glycol monoesters may be selected from the following partial list:

|                 |                                                                                |
|-----------------|--------------------------------------------------------------------------------|
| Acetic          | Methoxy propionic                                                              |
| Propionic       | Ethoxyethoxy acetic                                                            |
| Butyric         | Mono-2-ethylhexyl adipate                                                      |
| 2-ethyl butyric | Mono-C <sub>8</sub> Oxo sebatic                                                |
| Caproic         | C <sub>8</sub> -C <sub>20</sub> Oxo acids, including bottoms acids             |
| 2-ethylhexanoic | Acids derived from petroleum fractions by oxidation                            |
| Caprylic        | Pelargonic      Acids derived from alcohols and/or aldehydes by caustic fusion |
| Pelargonic      | Capric      Naphthenic acids                                                   |
| 25      Lauric  | Myristic      Glycolic acid                                                    |
| Stearic         | Oleic      Lactic acid                                                         |
|                 | Stearic      Hydroxystearic acid                                               |

This concept of the instant invention may be illustrated as follows:

#### EXAMPLE I

Preparation of n-butyl Carbitol-(CH<sub>2</sub>O-tripropylene glycol)<sub>4</sub> i. e.

- 35      n-C<sub>4</sub>H<sub>9</sub>(OCH<sub>2</sub>CH<sub>2</sub>)<sub>2</sub>O-(CH<sub>2</sub>OCH<sub>3</sub>H<sub>6</sub>OCH<sub>3</sub>H<sub>6</sub>O)<sub>4</sub>H
- The hemiformal of n-butyl Carbitol was made by heating 81.1 g. (1/2 mole) of the Carbitol with 15.1 g. (1/2 mole CH<sub>2</sub>O) of paraformaldehyde, 200 g. of heptane and 2 g. of NaHSO<sub>4</sub> at 65° C. for half an hour.
- 40      The polyformal of tripolypropylene glycol, i. e. TPG-CH<sub>2</sub>O-TPG-CH<sub>2</sub>O-TPG-CH<sub>2</sub>O-TPG was made by refluxing 384.5 g. (2 moles) of tripolypropylene glycol, 45.5 g. (1.5 moles CH<sub>2</sub>O) of paraformaldehyde, 200 g. of heptane and 3.2 g. of NaHSO<sub>4</sub> for 90 minutes at 89° to 104° C. The volume of the water layer was 28 cc. (theoretical is 27 cc.). To minimize simple formal formation the hemiformal of n-butyl Carbitol was added dropwise over a period of 70 minutes to the refluxing solution of the polyformal of tripolypropylene glycol. After the hemiformal was added refluxing at 100°-102° C. was continued for an additional 30 minutes. The volume of the water layer was now 37 cc. (theoretical is 36 cc.). The catalyst was removed by decanting. The mixture was then washed with three 100 cc. portions of 5% Na<sub>2</sub>CO<sub>3</sub> and two 100 cc. portions of water. After stripping off the solvent and unreacted material, the product boiling above 140° C. at .2 mm. (kettle temperature of 231° C.) gave the following inspections:

- 50      60      Viscosity, cs. at ° F.:  
 210 ----- 50.86 (235 SUS)  
 100 ----- 423.1  
 0 ----- 59,700

- 65      Viscosity index ----- 130  
 Pour point, ° F. ----- -25  
 Hydrogen combustion test: Carbon, 1.1 mgs.; varnish, 0.7 mg.

#### EXAMPLE II

- 70      Preparation of polyethylene glycol polyformal i. e., HO(CH<sub>2</sub>CH<sub>2</sub>O)<sub>6.4</sub>[CH<sub>2</sub>(OCH<sub>2</sub>CH<sub>2</sub>)<sub>6.4</sub>O]<sub>2</sub>H

This polyformal was made by heating 300 g. (1 mole) of polyethylene glycol of a molecular weight of about 300, 30 g. (1 mole CH<sub>2</sub>O) of paraformaldehyde, 200 g.

of heptane and 3.3 g. of  $\text{NaHSO}_4$  to  $98^\circ \text{C}$ . for two hours during which time 19.2 cc. of a water layer was collected (theoretical is 18 cc.). After cooling the heptane layer was separated. The polyformal layer was treated with 10% animal charcoal at  $115^\circ \text{C}$ . for 30 minutes and then suction filtered. The polyformal is compared below with the original polyethylene glycol 300.

|                                         | Polyethylene Glycol 300 | Polyformal of PEG-300 |
|-----------------------------------------|-------------------------|-----------------------|
| Viscosity, Cs. at $^{\circ}\text{F}.$ : |                         |                       |
| 210                                     | 5.68 (44.79 SUS)        | 36.40 (170.7 SUS)     |
| 100                                     | 34.24 (159.8 SUS)       | 290.7 (1343 SUS)      |
| Viscosity Index                         | 116                     | 132                   |
| Pour Point, $^{\circ}\text{F}.$         | +5                      | +30                   |
| Flash Point, $^{\circ}\text{F}.$        | 400                     | 360                   |
| Fire Point, $^{\circ}\text{F}.$         | 445                     | 460                   |

According to a second concept of the instant invention, the molecules set out by the type formulas above that have a free hydroxyl group may be further treated with formaldehyde and joined to another organic compound having a free alcoholic hydroxyl group. This series of compounds, all of which the grouping  $-(\text{formaldehyde-glycol})_x$ ,  $x$  being greater than 1, may be shown as follows; the common grouping being designated by "Z":

Alcohol-Z-formaldehyde-alcohol  
Alcohol-Z-formaldehyde-glycol monoester  
Alcohol-Z-formaldehyde-glycol monoether  
Glycol monoester-Z-formaldehyde-glycol monoester  
Glycol monoester-Z-formaldehyde-glycol monoether  
Glycol monoether-Z-formaldehyde-glycol monoether

By substituting a hydroxy acid monoester such as lactates and glycolates, another series of compounds may be prepared as follows:

Hydroxy monoester-Z-formaldehyde-hydroxy monoester  
Hydroxy monoester-Z-formaldehyde-alcohol  
Hydroxy monoester-Z-formaldehyde-glycol monoether  
Hydroxy monoester-Z-formaldehyde-glycol monoester

It will be seen that the above mentioned complex formals all are included under the generic formula:

A—(formaldehyde-glycol) $_x$ —formaldehyde—B  
or  
A—O—[CH<sub>2</sub>—O—(C<sub>n</sub>H<sub>2n</sub>O)<sub>y</sub>]<sub>x</sub>CH<sub>2</sub>—O—B

wherein A and B may be the same or different and are selected from the group consisting of organic radicals containing from 1 to 60 carbon atoms which corresponds to organic compounds containing a hydroxyl group that is alcoholic in nature and wherein  $x$  and  $n$  are whole numbers greater than 1 and  $y$  is 1 or more.

This concept of the invention may be further illustrated by the following examples:

### EXAMPLE III

Preparation of C<sub>13</sub> Oxo Alcohol-(CH<sub>2</sub>O-Tripropylene Glycol)<sub>3</sub>CH<sub>2</sub>O—C<sub>13</sub> Oxo Alcohol i. e.,



The central portion, i. e.,



of this polyformal was first made by refluxing 288 g. (1.5 moles) of tripropylene glycol, 30 g. (1 mole CH<sub>2</sub>O) of trioxymethylene, 300 g. of heptane and 5.5 g. of catalyst (NaHSO<sub>4</sub>) for 40 minutes at  $89^\circ \text{C}$ . to  $100^\circ \text{C}$ . The volume of water collected was 19 cc. (theoretical is 18 cc.). The reaction mixture was cooled to  $70^\circ \text{C}$ . at which point 200 g. (1 mole) of C<sub>13</sub> Oxo alcohol and 30 g. (1 mole CH<sub>2</sub>O) of trioxymethylene were added. The reaction mixture was then heated at reflux temperature  $90^\circ$ – $103^\circ \text{C}$ . for 30 minutes during which time 19.5 cc. (theory is 18 cc.) of water was collected.

The reaction product was decanted from the catalyst and then washed with 150 cc. of 10% Na<sub>2</sub>CO<sub>3</sub> solution

and finally with two 100 cc. portions of water. The material was then stripped free of the solvent and light ends. The material boiling above  $152^\circ \text{C}$ . at 0.3 mm. pressure and consisting of the 14–100% fraction had the following properties:

|                                         |                                                             |  |
|-----------------------------------------|-------------------------------------------------------------|--|
| Viscosity, cs. at $^{\circ}\text{F}.$ : |                                                             |  |
| 210                                     | 8.91                                                        |  |
| 100                                     | 56.67                                                       |  |
| 0                                       | 4657                                                        |  |
| 10                                      | 132                                                         |  |
| Viscosity index                         |                                                             |  |
| Pour point, $^{\circ}\text{F}.$         | —45                                                         |  |
| Flash point, $^{\circ}\text{F}.$        | 420                                                         |  |
| Fire point, $^{\circ}\text{F}.$         | 455                                                         |  |
| 15                                      | Hydrogen combustion test: Carbon, 1.3 mg.; varnish, 0.2 mg. |  |

The clean burning characteristics of this reaction product indicate that it would give essentially no octane requirement increase if it were used as an automotive 20 crankcase lubricant.

### EXAMPLE IV

Preparation of C<sub>13</sub> Oxo Alcohol-(CH<sub>2</sub>O-Tripropylene Glycol)<sub>2</sub>—CH<sub>2</sub>O—C<sub>13</sub> Oxo Alcohol

25 This complex formal which is similar to that prepared above was made to obtain a lower viscosity material. The C<sub>13</sub> Oxo alcohol (520 g., 2.6 moles), 117 g. of para-formaldehyde (3.9 moles CH<sub>2</sub>O), 200 g. of heptane and 3.1 g. (0.25% of NaHSO<sub>4</sub>) catalyst were heated to  $55^\circ \text{C}$ . for 45 minutes. To this hemiformal of C<sub>13</sub> Oxo alcohol was then added 500 g. (2.6 moles) of tripropylene glycol and the mixture heated to reflux. After three 30 hours the temperature had risen from  $95^\circ \text{C}$ . to  $118^\circ \text{C}$ . and 73 cc. of water had been collected. (The theoretical amount of water is 70.2 cc.) The material was light tan in color indicating that the small catalyst concentration (0.25%) was helpful in not causing excessive discoloration which occurs when the usual 1% catalyst is employed. The reaction product was separated from 35 the crystalline catalyst and washed with three 100 cc. portions of saturated Na<sub>2</sub>CO<sub>3</sub> solution and then with three 100 cc. portions of water before stripping of the heptane and small amount of water. The product boiling above  $153^\circ \text{C}$ . at 0.2 mm. mercury pressure and 40 consisting of the 6 to 100% fraction had the following properties.

|                                                             |                                 |         |
|-------------------------------------------------------------|---------------------------------|---------|
| Viscosity, cs. at $^{\circ}\text{F}.$ :                     |                                 |         |
| 210                                                         | 5.82                            |         |
| 100                                                         | 33.82                           |         |
| 50                                                          | 2286                            |         |
| 0                                                           | —40                             | 80,000+ |
| Viscosity index                                             |                                 | 125     |
| Pour point, $^{\circ}\text{F}.$                             | —50                             |         |
| Flash point, $^{\circ}\text{F}.$                            | 390                             |         |
| 55                                                          | Fire point, $^{\circ}\text{F}.$ | 430     |
| Hydrogen combustion test: Carbon, 0.8 mg.; varnish, 0.2 mg. |                                 |         |

### EXAMPLE V

60 Preparation of n-Butyl-(OC<sub>3</sub>H<sub>6</sub>)<sub>2</sub>O(CH<sub>2</sub>O-Polypropylene Glycol 150)<sub>2</sub>—CH<sub>2</sub>O—(OC<sub>3</sub>H<sub>6</sub>)<sub>2</sub>n-Butyl

The preparation of this complex formal was accomplished according to the description of Example IV.

The material obtained boiling above  $161^\circ \text{C}$ . at 0.3 mm. 65 had the following properties:

|                                  |                                 |       |
|----------------------------------|---------------------------------|-------|
| Viscosity at—                    |                                 |       |
| 210° F.                          | 3.72                            |       |
| 100° F.                          | 17.30                           |       |
| 70                               | 0                               | 591.7 |
| —40° F.                          | 12,220                          |       |
| Viscosity index                  |                                 | 116   |
| Pour point, $^{\circ}\text{F}.$  | —70                             |       |
| Flash point, $^{\circ}\text{F}.$ | 330                             |       |
| 75                               | Fire point, $^{\circ}\text{F}.$ | 345   |

The fraction of the product boiling above 188° C. at 0.2 mm. had the following properties:

|                   |        |
|-------------------|--------|
| Viscosity at—     |        |
| 210° F.           | 5.39   |
| 100° F.           | 29.46  |
| 0                 | 1709   |
| —40° F.           | 55,849 |
| Viscosity index   | 129    |
| Pour point, ° F.  | —60    |
| Flash point, ° F. | 350    |
| Fire point, ° F.  | 390    |

#### EXAMPLE VI

Preparation of C<sub>13</sub> Oxo Alcohol-(CH<sub>2</sub>O-Tripropylene Glycol)<sub>2,3</sub>-CH<sub>2</sub>O-C<sub>13</sub> Oxo Alcohol

Two moles C<sub>13</sub> Oxo alcohol, 3.7 moles of formaldehyde, as paraformaldehyde, and 2.3 moles of tripropylene glycol were admixed with 300 g. heptane and 1.5 g. of sodium acid sulfur. The mixture was heated to reflux temperature until the theoretical water was evolved. The product was then decanted from the catalyst and washed with 100 cc. portions of sodium carbonate three times; it was then washed twice with 100 cc. portions of water and then filtered. The material was then stripped to 176° C. vapor temperature at 10 mm. The product had the following properties:

|                   |                   |
|-------------------|-------------------|
| Viscosity at—     |                   |
| 210° F.           | 8.06 (52.6 SUS)   |
| 100° F.           | 47.81 (221.3 SUS) |
| 0                 | 3491              |
| —40° F.           | 110,000+          |
| Viscosity index   | 136               |
| Pour point, ° F.  | —50               |
| Flash point, ° F. | 425               |
| Fire point, ° F.  | 460               |

#### EXAMPLE VII

Preparation of C<sub>13</sub> Oxo Alcohol-CH<sub>2</sub>O(Triethylene Glycol-CH<sub>2</sub>O)<sub>2</sub>-C<sub>13</sub> Oxo Alcohol

400 g. of C<sub>13</sub> Oxo alcohol and 67.2 g. of formaldehyde was admixed and heated with 2.4 g. of NaHSO<sub>4</sub> in the presence of 240 g. of heptane. The mixture was then heated to 55° F. for approximately 25 minutes. To this mixture 300 g. of triethylene glycol was added and this mixture heated to 113° C. for approximately one hour. At this point 33.6 g. additional formaldehyde was added to the reacting mixture. This mixture was then heated to 115° C. for an additional hour. At the end of this period 60 g. of water had been removed (54 g. theoretical).

This product was purified in the manner similar to that of Example VI above and stripped to 210° C. vapor temperature at 9.0 mm. pressure.

This product had the following properties:

|                   |                   |
|-------------------|-------------------|
| Viscosity at—     |                   |
| 210° F.           | 6.34 (46.9 SUS)   |
| 100° F.           | 33.87 (158.2 SUS) |
| 0                 | 16,049            |
| —40° F.           | 44,306            |
| Viscosity index   | 142               |
| Pour point, ° F.  | —60               |
| Flash point, ° F. | 430               |
| Fire point, ° F.  | 470               |

#### EXAMPLE VIII

Preparation of C<sub>13</sub> Oxo Alcohol—O(CH<sub>2</sub>O—Pantanediol-1,5)<sub>3</sub>-CH<sub>2</sub>—O—C<sub>13</sub> Oxo Alcohol

This product was prepared as described in Example VII above except that the glycol was pentanediol-1,5 instead of triethylene glycol. The product was stripped to a vapor temperature of 182° C. at 10 mm. pressure.

The properties of this product are as follows:

|                   |                   |
|-------------------|-------------------|
| Viscosity at—     |                   |
| 210° F.           | 12.28 (67.4 SUS)  |
| 100° F.           | 75.56 (349.3 SUS) |
| 0                 | 4,035             |
| —40° F.           |                   |
| Viscosity index   | 143               |
| Pour point, ° F.  | —35               |
| Flash point, ° F. | 440               |
| Fire point, ° F.  | 485               |

15 The complex formals as described herein may serve as the lubricant base for grease compositions. These synthetic lubricants may be thickened to stable grease structures with conventional grease forming soaps such as lithium soaps of high molecular weight substantially saturated fatty acid, the n-acyl p-amino phenols, silica gels, treated bentonites and the like. Oxidation inhibitors, rust inhibitors, tackiness agents and other grease addition agents may be added to the complex formal greases. The soap complexes known to the art made by using low molecular weight acid salts may also be used in preparing these grease compositions. If desired the complex formals of this invention may be blended with mineral oil or other synthetic lubricants such as simple bis-formals, complex esters, di-esters, phosphates, siloxanes, silicates, phosphonates and the like and a grease composition which incorporates the desirable characteristics of the blends may be prepared by conventional techniques.

20 The following illustrates the procedures used in preparing the grease compositions generally described above:

#### Formulation

25 20.0 wt. percent lithium fatty acid soaps (Litholite A)<sup>1</sup>  
1.0 wt. percent phenyl alpha-naphthylamine  
79.0 wt. percent complex formal, i. e., C<sub>13</sub> Oxo-(CH<sub>2</sub>O-tripropylene glycol)<sub>3</sub>-CH<sub>2</sub>O-C<sub>13</sub> Oxo alcohol

#### Preparation

40 A very good dispersion of the soap in the synthetic oil was obtained by heating the soap and oil to 450° F. with stirring. During the early stages of heating the mass swelled. The phenyl alpha-naphthylamine was added and the mass was pan cooled. The resulting product had an excellent grease structure and had a dropping point of 379° F.

45 To summarize briefly, this invention relates to new compositions of matter which have outstanding utility as synthetic lubricating compositions. The materials contemplated may be broadly described as being complex formals of organic materials containing at least one hydroxyl group that is alcoholic in nature. By complex formal is meant materials containing more than 2 formal linkages. The structure of the formals of invention may be described as one corresponding to the formula:



50 where x and n are whole numbers greater than 1 and y has a value of 1 or more. In this formula A and B are organic radicals containing from 1 to 60 carbon atoms which are derived from organic materials containing at least one hydroxyl group that is alcoholic in nature. A and B may be alike or different and the total number of carbon atoms in the molecule should be between about

55 20 and 130, preferably between about 25 and 100. The compounds that are especially preferred and that are considered to be the preferred embodiment of this invention are those materials that have a kinematic viscosity at 210° F. within the range of from 2 to 60 centistokes, an ASTM pour point of at least as low as 35° F., and a flash point of at least 300° F.

60 The formals of this invention are useful as plasticizers,

75 <sup>1</sup> Lithium stearate, see Foote Prints (published by Foote Mineral Company, Philadelphia), volume 21, No. 1 (1949), page 25.

solubilizers, grease bases, insecticides, weed killers, rust preventives, solvents, dewaxing aids, detergents, and as raw materials for many other industrial applications, such as household detergents, fumigants, etc. These new synthetic lubricating oils may be admixed with other lubricating oils, naturally occurring or synthetic, either as concentrates or as finished blends. They are compatible and may be blended with the well known lubricant addition agents such as viscosity index improvers, pour point depressors, detergents, rust inhibitors, antioxidants, and the like.

What is claimed is:

1. As a synthetic lubricant, a complex formal having an ASTM pour point below about 35° F., a flash point above about 300° F., and a kinematic viscosity at 210° F. within the range of from 2 to 60 centistokes, said formal corresponding to the formula



wherein A and B are selected from the group consisting of hydrocarbon and substituted hydrocarbon radicals containing from 1 to 60 carbon atoms wherein x and n are integers having a value of at least 2 and y is an integer having a value of at least 1, the total number of carbon atoms in the molecule being between 20 and 130.

2. A synthetic lubricant according to claim 1 wherein A is derived from monohydric alcohol and wherein B is derived from a glycol.

3. A synthetic lubricant according to claim 1 wherein A and B are organic radicals derived from C<sub>8</sub> to C<sub>20</sub> branched chain alcohols and wherein n, y and x are 3.

4. As a synthetic lubricant, a complex formal having the formula



wherein A and B are organic radicals derived from C<sub>8</sub> to C<sub>20</sub> alcohols and wherein x and n are numbers having the value of 2 or more and y is an integer having a value of at least 1, said formal being formed by reacting together x.y moles of a glycol with x+1 moles of formaldehyde and 2 moles of an alcohol containing from 8 to 20 carbon atoms, said formal having an ASTM pour point below about +35° F., a flash point above about 300° F., and a viscosity at 210° F. within the range of from 2 to 60 centistokes, the total number of carbon atoms in the molecule being between about 25 to 100.

5. A synthetic lubricant according to claim 4 wherein

said alcohol is a highly branched chain aliphatic alcohol of 8 to 20 carbon atoms.

6. A synthetic lubricant according to claim 4 wherein said glycol is tripropylene glycol.

7. A synthetic lubricant according to claim 4 wherein said glycol is a polyethylene glycol.

8. A synthetic lubricant according to claim 4 wherein said alcohol is a highly branched chain aliphatic alcohol of 13 carbon atoms alcohol and wherein x, n, and y are 3.

9. A synthetic lubricant according to claim 4 wherein said alcohol is an ether alcohol, wherein said glycol is a propylene glycol of a molecular weight of about 150 and wherein x is 2.

10. A synthetic lubricant according to claim 4 having an ASTM pour point of below -15° F., a flash point in excess of 350° F. and viscosity at 210° F. of from 2.6 to 13.0 centistokes.

11. As a synthetic lubricant, a complex formal of the formula



wherein A and B are selected from the group consisting of hydrocarbon and substituted hydrocarbon radicals containing from 1 to 60 carbon atoms and wherein x and n

25 are numbers having the value of at least 2 and wherein y is a number of at least 1 thickened to a grease consistency with a lithium soap of a high molecular weight fatty acid, said complex formal having an ASTM pour point below about +35° F., a flash point above about 300° F., and a viscosity at 210° F. within the range of from 2-60 centistokes, the total number of carbon atoms in said formal being between about 20 to 130.

#### References Cited in the file of this patent

##### UNITED STATES PATENTS

|              |               |               |
|--------------|---------------|---------------|
| 2,350,350    | Gresham       | June 6, 1944  |
| 2,379,703    | Geltner       | July 3, 1945  |
| 2,397,602    | Gresham       | Apr. 2, 1946  |
| 40 2,436,347 | Zimmer et al. | Feb. 17, 1948 |
| 2,473,994    | Gresham       | June 21, 1949 |
| 2,594,341    | Owen et al.   | Apr. 29, 1952 |

##### OTHER REFERENCES

45 Wender and Orchin: Critical Review of Chem. of Oxo-Synthesis, Bur. of Mines, R. I. 4270, June 1948, pages 6 and 9.